

# United States Patent [19]

Rubin

[11] 3,867,489

[45] Feb. 18, 1975

[54] **METHOD OF PRODUCING AN  
OXIDATION-RESISTANT UO<sub>2</sub> FUEL BODY**

[75] Inventor: **Jack A. Rubin, Encino, Calif.**

[73] Assignee: **The United States of America as  
represented by the United States  
Atomic Energy Commission,  
Washington, D.C.**

[22] Filed: **July 17, 1962**

[21] Appl. No.: **210,880**

[52] U.S. Cl. .... **264/0.5, 252/301.1 R**

[51] Int. Cl. .... **G21c 20/00**

[58] **Field of Search** ..... 204/154.2, 193.2; 264/0.5;  
252/301.1 R

## [56] References Cited

### UNITED STATES PATENTS

2,816,042 12/1957 Hamilton ..... 106/565  
2,818,605 1/1958 Miller ..... 106/55

### FOREIGN PATENTS OR APPLICATIONS

874,964 8/1961 Great Britain ..... 106/565

### OTHER PUBLICATIONS

AEC Report, WAPD-MRP-68, June 1959, pp. 80-82.

AEC Report, WAPD-MRP-78, Aug. 1957, pp. 57 and  
63.

J. of American Ceramic Soc., vol. 35, No. 5 May  
1952, pp. 107-113.

Nuclear Power, May 1959, pp. 86-88.

AEC Report, TID-7546 (Book 2), Nov. 1957, pp. 532  
and 533.

*Primary Examiner*—Carl D. Quarforth

*Assistant Examiner*—Roger S. Gaither

*Attorney, Agent, or Firm*—John A. Horan; Frederick  
A. Robertson

## EXEMPLARY CLAIM

1. A method of forming a UO<sub>2</sub> fuel body resistive to  
oxidative attack, which comprises mixing UO<sub>2</sub> and a  
ceramic oxide of relatively low thermal neutron ab-  
sorption cross section, adding to the resulting mixture  
a small amount of a compound selected from the class  
consisting of alkali metal halides, and alkaline earth  
metal halides, and then forming a fuel body of the re-  
sulting composition.

**9 Claims, No Drawings**

## METHOD OF PRODUCING AN OXIDATION-RESISTANT UO<sub>2</sub> FUEL BODY

My invention relates to a method of producing an oxidation-resistant UO<sub>2</sub> fuel body, and more particularly to a method of producing a fuel body in which UO<sub>2</sub> is contained within the grains of a ceramic matrix.

Uranium dioxide fuel elements have been made in mixtures with ceramic moderator and ceramic structural compositions. UO<sub>2</sub> is radiation stable and may go to high fuel burnups. However, it is readily oxidized in air and is lost by subsequent volatilization. This presents a serious limitation to the use of unclad ceramic UO<sub>2</sub> fuel bodies, especially in gas-cooled reactors. It has been observed that UO<sub>2</sub> compositions prepared by mechanical mixing and hot pressing have UO<sub>2</sub> positioned at the grain boundaries of the matrix material; this probably subjects the fuel body to greater oxidative attack than would be experienced by protectively encasing the UO<sub>2</sub> grains within grains of the matrix material. Such encasement has been accomplished by chemical coprecipitation of UO<sub>2</sub> and BeO, but this has entailed the handling of large volumes of solution, and there are other inconveniences and costs associated with handling of solutions.

An object of my present invention is, therefore, to provide an improved method of producing an oxidation-resistant UO<sub>2</sub> fuel body.

Another object is to provide a method of encasing UO<sub>2</sub> fuel within the grains of a ceramic matrix material to thereby improve its oxidation resistance.

Another object is to provide such a method which does not involve the handling of large volumes of solution.

A further object of my invention is to provide an improved method of forming a UO<sub>2</sub>—BeO fuel body wherein the UO<sub>2</sub> is contained within the BeO matrix.

A still further object is to provide an additive which will promote the encasement of UO<sub>2</sub> within a ceramic fuel body matrix.

Still other objects and advantages of my invention will become apparent from the following detailed description and the appended claims.

In accordance with my present invention an oxidation-resistant UO<sub>2</sub>-ceramic fuel body may be prepared by mixing UO<sub>2</sub> and ceramic powders, and adding thereto a small amount of a substance which forms a low melting liquid phase at or below the sintering temperature of the matrix. Use of the additive overcomes the poor sintering and oxidation characteristics of prior UO<sub>2</sub>-ceramic compositions apparently caused by pinning of the ceramic oxide grains by the UO<sub>2</sub> grains lodged at the grain boundaries; such pinning prevents any ceramic oxide grain growth around the UO<sub>2</sub>.

The mechanism for grain growth may involve the following. As the refractory ceramic oxide powder, comprising the ceramic matrix, grows into grains during the sintering process, the presence of a liquid phase caused by my additives probably acts as a media for material transport of the ceramic matrix allowing the ceramic grains to grow around the UO<sub>2</sub> grains, thus enclosing them and protecting them against subsequent loss when exposed to an oxidizing environment. Without the presence of this liquid phase-forming additive the UO<sub>2</sub> grains are pushed into the grain boundaries of the matrix during sintering where they are subject to easy oxidative attack. Upon prolonged sintering, the liquid phase disappears because of volatilization of the liquid

phase and/or incorporation of the phase into the matrix as a solid solution.

I have found that halides of the alkali metals (e.g., Na, Li), the alkaline earth metals (e.g., Mg, Sr, Ba), and the rare earth metals (e.g., Y, La) are satisfactory additives for use in my process. CaO is also satisfactory, this oxide forming a low melting eutectic, for example CaO—BeO eutectic is in the liquid phase at approximately 1,300° C. The fluoride salts of the foregoing metal halides are preferred, these being stable and low melting. MgF<sub>2</sub> is a particularly satisfactory composition; BeO may dissolve in molten MgF<sub>2</sub> at or below the sintering temperature of the ceramic matrix, which allows material transport of BeO around the grains of UO<sub>2</sub>, unpinning boundaries and allowing growth to continue by mass transfer of BeO.

Although the concentration of the additive may satisfactorily vary, generally only a small amount need be added to secure effective results. For example, approximately 0.1–1 wt. % is suitable, while about 0.25 wt. % is preferred. The powders may be mechanically mixed in weight concentrations and then blended by conventional means, such as ball-milling, mulling, wet mixing, and the like. After homogenization and dispersion the powders are formed into a ceramic body by methods known to the art, for example hot pressing, sintering, and the like.

The term "ceramic matrix material" is used herein to cover the refractory metal oxides which are customarily used in the nuclear reactor art with UO<sub>2</sub> in fuel bodies. For example, fuel-moderator bodies are formed with BeO, and non-moderating fuel bodies are formed with Al<sub>2</sub>O<sub>3</sub> and MgO as structural materials, these latter being refractory oxides of relatively low thermal neutron absorption cross section. UO<sub>2</sub>—BeO fuel bodies have also been formed containing a small amount (e.g., 1 wt. %) of a third oxide such as MgO or Y<sub>2</sub>O<sub>3</sub> to enhance the high temperature ductility of BeO and to improve the grain characteristics of BeO. The ceramic oxide is the major constituent in such fuel and fuel-moderator compositions. The concentration of uranium in the body may satisfactorily vary over a wide range; it will be determined by reactor design considerations and by enrichment of the uranium with respect to the fissionable U-235 isotope. For example, in a UO<sub>2</sub>—BeO fuel body using fully enriched uranium (approx. 93% U-235), the UO<sub>2</sub> will vary between about 5 to 15 Wt. %.

The UO<sub>2</sub> does not have to be added as such, but may be added as any uranium compound which can be decomposed to produce UO<sub>2</sub>, for example uranyl nitrate. Similarly, the matrix ceramic may be added in the form of a chemical compound which can be readily decomposed to the oxide, for example beryllium nitrate which can be decomposed to BeO during any sintering or hot pressing steps. The additive also can be formed by suitable chemical reaction rather than the direct addition of the necessary compound. For example, Na<sub>2</sub>BeF<sub>4</sub> reacts with MgO in a BeO-1% MgO fuel composition thereby producing the desired MgF<sub>2</sub> liquid. If fluorine were present as an impurity in BeO, it would react with MgO forming MgF<sub>2</sub> liquid.

It is generally preferred to form the fuel body in a hot pressing operation. The mixed powders are placed in a die of selected fuel body shape, and the assembly placed in a chamber having a non-oxidizing atmosphere. The term "non-oxidizing" is intended to em-

brace reducing atmospheres, such as hydrogen and carbon monoxide; vacuum; and inert gas atmospheres such as argon. The time-temperature-pressure relationship for the hot pressing step may satisfactorily vary while producing suitable fuel bodies. I find that a generally satisfactory temperature range is about 1,400°-1,800° C, a satisfactory pressure range about 2,000-6,000 psi, and the time may vary from about 2 to 8 hours. The preferred hot pressing conditions for UO<sub>2</sub>-BeO comprise heating the fuel body in an argon atmosphere at a temperature of about 1,600° C, at about 2,000 psi for about 4 hours.

The following examples are offered to illustrate my invention in greater detail.

#### EXAMPLE I

125 grams of a mixture of finely divided powders consisting of 94.25 wt.% beryllium oxide, 5 wt.% uranium dioxide (approx. 93% U-235), and 0.75 wt.% of calcium fluoride are thoroughly mixed together. To this mixture is added 100 ml. distilled water to produce a suspension which has a paint-like consistency. This suspension is then placed in a rubber lined ball-mill and homogenized for a period of 4 hours. The suspension is dried in a conventional spray dryer producing a homogeneous, granular, free-flowing powder.

This powder is then placed in a high strength graphite die. The die with its contents is placed in an argon atmosphere, and heated at the approximate rate of 500° C per hour beginning at the ambient temperature. When a temperature of 800° C is reached, a pressure of 2,000 psi is applied to the die. The heating is continued at the same rate until a temperature of 1,600° C is reached, meanwhile holding the pressure constant. The temperature is then held constant at 1,600° C for 4 hours, during which time the pressure remains at 2,000 psi. At the end of this time the pressure is released and the die is allowed to slowly cool to room temperature.

The resulting ceramic body is approximately 99% of theoretical density, and possesses a minimum transverse breaking strength of 20,000 psi at room temperature. This body loses no more than 0.1% of its weight when exposed to air flowing at 75 cfm for 4 hours at 1,650° C, which attests to its excellent oxidation resistance.

#### EXAMPLE II

The same as Example I except that the ceramic matrix is Al<sub>2</sub>O<sub>3</sub> and the salt is MgF<sub>2</sub>. This body also possesses excellent resistance to oxidative attack.

The above examples are only illustrative rather than restrictive of my invention, which should be understood to be limited only as is indicated in the appended claims.

I claim:

1. A method of forming a UO<sub>2</sub> fuel body resistive to oxidative attack, which comprises mixing UO<sub>2</sub> and a ceramic oxide of relatively low thermal neutron absorption cross section, adding to the resulting mixture a small amount of a compound selected from the class consisting of alkali metal halides and alkaline earth metal halides, and then forming a fuel body of the resulting composition.
- 10 2. A method of forming a fuel body which comprises mixing UO<sub>2</sub> and a refractory oxide of relatively low thermal neutron absorption cross section selected from the class consisting of BeO, BeO-MgO, MgO, and Al<sub>2</sub>O<sub>3</sub>, adding to the resulting mixture a small amount of a compound selected from the class consisting of alkali metal halides and alkaline earth metal halides, and then forming a ceramic fuel body of the resulting composition.
- 15 3. A method of forming a UO<sub>2</sub> fuel body which comprises mixing UO<sub>2</sub> and BeO powders, adding to said mixture a small amount of a compound selected from the class consisting of alkali metal halides and alkaline earth metal halides, and then forming a UO<sub>2</sub>-BeO fuel body of the resulting mixture.
- 20 4. The method of claim 3 wherein approximately 0.1-1 wt. % of the last-named additive is added to said UO<sub>2</sub>-BeO fuel composition.
5. The method of claim 3 wherein said UO<sub>2</sub>-BeO fuel body is formed by hot pressing said resulting mixture in a non-oxidizing atmosphere.
- 25 6. A method of forming a UO<sub>2</sub>-BeO fuel body, which comprises mixing UO<sub>2</sub> and BeO powders, adding to the resulting mixture approximately 0.1-1 wt. % of an alkaline earth metal fluoride, and then hot pressing the resulting composition in a non-oxidizing atmosphere to produce the UO<sub>2</sub>-BeO fuel body.
- 30 7. The method of claim 6 wherein said hot pressing is conducted under the approximate conditions of 1,400°-1,800° C, 2,000-6,000 psi, and 2 to 8 hours in an inert gas atmosphere.
- 35 8. The method of claim 6 wherein said UO<sub>2</sub> comprises approximately 5-15 wt. % of the fuel body composition.
- 40 9. A method of forming a UO<sub>2</sub>-BeO fuel body which comprises forming a powder mixture consisting essentially of 5-15 wt. % UO<sub>2</sub>, approximately 0.25 wt. % alkaline earth metal fluoride, and the remainder BeO, forming an aqueous suspension of the resulting mixture, drying the resulting suspension, placing the dried powders in a die in an inert gas atmosphere, and then hot pressing said powders under the approximate conditions of 1,600° C and 2,000 psi for 4 hours.

\* \* \* \* \*